

May 2, 1944.

J. C. MAYS

2,347,920

## ABRASIVE WHEEL

Filed March 27, 1941

Fig. 1.



Fig. 2.



Fig. 3.



### *Inventor:*

JAMES C. MATS

by W. Doley  
Attorney

## UNITED STATES PATENT OFFICE

2,347,920

## ABRASIVE WHEEL

James C. Mays, Niagara Falls, N. Y., assignor to  
The Carborundum Company, Niagara Falls,  
N. Y., a corporation of Delaware

Application March 27, 1941, Serial No. 385,407

12 Claims. (Cl. 51—309)

This invention relates to metal-bonded abrasive articles. More particularly, the invention relates to thin metal-bonded abrasive articles, such as cut-off wheels, in which the bond metal is deposited in situ electrolytically.

One of the objects of my invention is to provide thin abrasive wheels, such as cut-off wheels, in which at least the outer working portion of the wheel is composed wholly of abrasive particles bonded with electro-deposited metal, thereby producing abrasive articles of novel characteristics.

In making abrasive articles of certain types, the use of very hard abrasive such as diamond is desirable. Diamond abrasive is, however, so extremely expensive that, while the ordinary commercial abrasives are sold for about five cents per pound, diamond abrasive sells for around two thousand dollars per pound. It will be obvious, therefore, that in commercial practice when using diamond abrasive in the manufacture of abrasive articles the quantity of abrasive which can economically be used will be very small, and that the diamond abrasive particles must be very firmly held in the matrix of bond metal so that most or all of their potential usefulness as an abrasive is exhausted before they are released by the bond metal.

I have found that abrasive particles disposed in a single layer can be firmly and permanently held by a single layer of metal electro-deposited in situ about them so that the abrasive particles are embedded in a matrix of such metal. The abrasive particles are held so firmly that the resulting structure makes a very efficient cut-off wheel for use on even the hardest materials.

The invention will be more readily understood by reference to the accompanying drawing, in which Fig. 1 is a view in plan of a cut-off wheel made in accordance with the present invention.

Fig. 2 is an enlarged fragmentary sectional view of a cut-off wheel of the type shown in Fig. 1, the view being taken along the line 2—2, in Fig. 1.

The cut-off wheel shown in Fig. 1 consists of a thin disc of electro-deposited metal, in the outer portion of which are embedded abrasive particles 2, said abrasive particles being arranged in a single layer in an annulus concentric with the disc. The center of the disc is provided with an arbor hole 3. Disc 1 is made with its thickness approximately that of the diameter of the largest abrasive particles in the wheel, so that the abrasive particles have their outer surfaces lying substantially in the planes of the side faces of disc 1.

By suitably removing small amounts of electro-deposited metal from the side faces of the disc 1, the abrasive particles may be exposed on both side faces of the cut-off wheel, as shown in Figs. 1 and 2.

In Figure 3, which is a fragmentary sectional view taken along the line 3—3 in Fig. 1, is shown the structure of a cut-off wheel of the type described. As shown, abrasive grains 2 are firmly held in a matrix composed of electro-deposited metal 1, but with points exposed on opposite sides of the matrix.

The apparatus illustrated in Figure 2 is designed for the manufacture of thin abrasive wheels, such as cut-off wheels, covered by the present invention, by electro-deposition of metal on abrasive particles. By the use of this apparatus a cut-off wheel can be made which is the approximate thickness of the diameter of the largest abrasive particles in the wheel. In Figure 2 a vessel 4 of non-conducting material such, for example, as glass, is used. Supported on the bottom of vessel 4 and centered by ring 5 is a plate 6 also of insulating material, such as a phenolic resin, in which is embedded a circular disc 7 of metal, such as copper, having a centrally located hole 8 therethrough. Extending partially into hole 8 is an insulating tube 9 within which is a wire 10 by which an electrical connection may be made to disc 7 through spring contact 11 attached to wire 10 and pressing against the sides of hole 8 in disc 7. Suspended from the upper edge of vessel 4 is an anode 12 of circular cross-section.

In the use of the apparatus shown in Figure 2, disc 7 is coated with a material such, for example, as a thin electro-deposited layer of lead, which will act as a parting layer, and is then placed in cell 4 and assembled with tube 9 and electrical connections 10 and 11. Since in making cut-off wheels it is usually unnecessary and when using costly abrasives such as diamond it is undesirable to have abrasive throughout the wheel, only the wheel rim contains abrasive. This is provided for in my invention by sliding over spacing washer 13 on tube 9 a cylindrical, non-conducting tube 14 which is allowed to rest on disc 7 thus leaving exposed a peripheral ring 15 of disc 7 of the desired size, the cell 4 having already been filled with plating solution. Abrasive particles are then introduced at the surface of the electrolyte in cell 4 around tube 14 and allowed to fall on the exposed portion 15 of disc 7, care being taken to obtain a uniformly distributed deposit of abrasive. Tube 14 is then

removed and plating carried out until the abrasive particles are covered with metal. Plating is then discontinued and the apparatus disassembled. The abrasive containing layer may be readily peeled off because of the parting layer previously placed on disc 7. After flattening, if necessary, the metal disc may be treated with acid to dissolve from the wheel sufficient metal to leave abrasive particles exposed on both side faces.

By the above-described method cut-off wheels much thinner than those obtainable by other methods may be produced. This is because of the fact that the electro-deposited metal bond is much stronger than bonds obtained by such methods as sintering. When suitable abrasive is used they are capable of use in cutting costly materials such as gems, quartz crystals, hard metal carbides and the like. It will be obvious that thicker wheels may be produced by supplying additional abrasive as the plating is continued so that the wheels may be of any desired thickness.

Any desired abrasive may be used in the abrasive wheels disclosed herein, but the wheel of the present invention is particularly advantageous when used with diamond abrasive, the high cost of which necessitates a very firm bonding of the abrasive particles so that the valuable abrasive is not pulled out nor dislodged. Moreover, various metals and alloys such as copper, brass, silver may be electro-deposited as a bond for the abrasive though in general, it may be desirable to use harder metals and alloys, such as nickel or chromium.

It will be obvious that modifications may be made in the abrasive wheel disclosed, and I therefore do not wish to be limited to the precise structure of the abrasive wheel described but only by the scope of the appended claims.

I claim:

1. In an abrasive cut-off wheel, a thin disc of electrolytically deposited metal, abrasive grains supported in said disc substantially all said grains extending therethrough so that a portion 45

of each grain is exposed at each of the radial faces of the disc.

2. An abrasive cut-off wheel as set out in claim 1 in which the electrolytically deposited metal is nickel.

3. An abrasive cut-off wheel as set out in claim 1 in which the electrolytically deposited metal is chromium.

4. An abrasive cut-off wheel as set out in claim 1 in which the electrolytically deposited metal is copper.

5. In an abrasive cut-off wheel, a thin disc of electrolytically deposited metal, abrasive grains supported in an annular peripheral band in said disc, substantially all of said grains extending therethrough so that a portion of each grain is exposed at each of the radial faces of said disc.

6. An abrasive cut-off wheel as set out in claim 5 in which the electrolytically deposited metal is nickel.

7. An abrasive cut-off wheel as set out in claim 5 in which the electrolytically deposited metal is chromium.

8. An abrasive cut-off wheel as set out in claim 5 in which the electrolytically deposited metal is copper.

9. A thin cut-off wheel consisting of a thin disc of electrolytically deposited metal having abrasive grains substantially uniformly distributed therethrough, the electrolytically deposited metal directly contacting the surfaces of the abrasive grains, a portion of said grains being exposed on both the radial surfaces and on the peripheral surface of the disc.

10. A thin cut-off wheel as set out in claim 9 in which the electrolytically deposited metal is nickel.

11. A thin cut-off wheel as set out in claim 9 in which the electrolytically deposited metal is chromium.

12. A thin cut-off wheel as set out in claim 9 in which the electrolytically deposited metal is copper.

JAMES C. MAYS.